

F. GIOLITTI.  
PROCESS FOR MANUFACTURING STEEL PLATES.  
APPLICATION FILED SEPT. 6, 1906.

1,024,770.

Patented Apr. 30, 1912.



*Witnesses:*

L. C. Badeau.  
H. J. Penney

*By his Attorney,*

*Inventor:*

Federico Giolitti,  
F. A. Richards

# UNITED STATES PATENT OFFICE.

FEDERICO GIOLITTI, OF ROME, ITALY, ASSIGNOR TO SOCIETA ANONIMA ITALIANA GIO.  
ANSALDO ARMSTRONG & CO., OF GENOA, ITALY, A CORPORATION OF ITALY.

## PROCESS FOR MANUFACTURING STEEL PLATES.

1,024,770.

Specification of Letters Patent. Patented Apr. 30, 1912.

Application filed September 6, 1906. Serial No. 333,408.

*To all whom it may concern:*

Be it known that I, FEDERICO GIOLITTI, doctor of chemistry, a subject of the King of Italy, and a resident of Rome, Italy, have 5 invented a certain new and useful Process for Manufacturing Steel Plates, of which the following is a specification.

This invention relates to a process for manufacturing armor plates or other objects made of steel composed of either superficial or deep successive zones in steels of different composition, not only as regards the proportion of carbon contained but also as regards the presence in some of them of 10 foreign metals and as regards the proportions in which these metals enter into the composition. This latter varies gradually in passing from one zone to another.

The accompanying drawing illustrates 20 diagrammatically a steel plate after treatment according to the present invention.

The result in question is obtained by submitting the mass of homogeneous steel (either ordinary carbon steel or a special 25 ternary, quaternary or like steel) to the action of suitable granular mixtures containing the metal it is desired to introduce into the steel, such as principally chromium, nickel, tungsten, molybdenum, vanadium, 30 and sometimes silicon and uranium in a free state or in a state of readily disassociated combination, which as is hereinafter stated varies from one preparation to the other as well as from one phase to the other of the 35 same preparation. These granular mixtures ought to be strongly compressed against one or both surfaces of the plate or other article to be treated.

For each given composition of the homogeneous steel which forms the mass under 40 manipulation as well as for one or more of the given metals contained in the mixture employed, there exists a determined interval or range of temperature, which depends 45 strictly on the position of the critical intervals of the homogeneous steel itself and on the nature of the metals employed. It is in 50 this interval that takes place the diffusion of the metal or metals contained in the mixture compressed against the surfaces of the 55 mass of steel toward the interior of this mass itself. The interval of temperature referred to above which is the most suitable for obtaining the diffusion in question, is comprised between the temperature of the

highest critical point of the steel employed and a temperature near its point of fusion.

The depth to which the metal contained in the granular mixture extends into the homogeneous mass of steel submitted to such an 60 operation depends above all on the length of the operation; but even by considerably prolonging this duration a very deep or gradual diffusion would not be obtained in 65 the greater number of cases if the temperature were always maintained constant from the beginning of the operation until the end.

In the drawing, representing the bar of treated material, the face *a* represents the bar unaltered while the other face *b* indicates the zone of treatment that extends into 70 the middle and is graduated in composition.

The constancy of the temperature—a condition which would be very useful if a certain concentration as regards the foreign 75 metal introduced had not been surpassed and if a great homogeneousness of concentrating for a given zone of the plate had to be obtained—prevents a very definite given limit of concentration being surpassed, because if 80 this latter is increased there is produced a displacement of the critical intervals and consequently of the interval of temperature in which the diffusion can be effected. It results that at a certain moment the temperature maintained constant is no longer comprised in this interval and consequently the 85 passage of the metal of the mixture to the mass under treatment is no longer effected and the diffusion is effected only at the interior of the mass until the concentration is 90 suitably lowered owing to the interior diffusion referred to. It will then generally be advisable to suitably alternate the reduction and the increases of temperature in 95 limits which can easily be determined for each case and which generally ought to determine the beginning and the ending of the critical intervals.

The product of the treatment referred to 100 above will consist of a heterogeneous mass of steel, the composition of which varies in the various zones or layers according to the composition of the microconstruction of the homogeneous steel started with, the composition of the granular mixture employed and the fixed or variable conditions of temperature in which the operation is effected. For example, if a start is made with an ordinary homogeneous carbon steel ingot and 110

if a granular mass containing only one metal is used for the treatment and compressed against only one face of the ingot, the result will be (beginning with the surface which has been submitted to the operation) a block formed of a ternary steel in which the proportion of the characteristic metal decreases toward the interior of the block until at a certain depth this temper is reduced to zero. From this moment the ingot will still be formed of the same primitive carbon steel which may have (as well as the ternary zone) the same initial proportion of carbon or a different proportion according as the granular mass did not contain active substances or was more or less rich in carbon or metallic oxides. As example a steel carbon plate (0.1 to 0.2 per cent. of carbon) may be taken, maintained in contact with a mixture of wolframic acid or of substances suitably "carbonaceous" or nitrogenous compressed against one of its surfaces at a temperature near that of fusion. As an example of such nitrogenous substances may be mentioned: charcoal 50%, bone-black 20%, carbonate of barium 25% and ferrocyanid of potassium 5%. In this case the preceding operation must be followed by a superficial decarbonization obtained by means of heating in contact with the mixtures of ordinary metallic oxides. On the contrary if a start is made with a ternary homogeneous steel ingot (for example, a chrome steel with 2 to 4 per cent. of chrome) the final product would have a similar structure to that of the preceding ingot but the layer of ternary steel would be substituted by a layer of quaternary steel, while the rest of the mass would still be ternary steel. In the case just mentioned by employing a mixture of the preceding case the quaternary layer will consist of chrome steel and wolfram steel. The procedure is followed in a similar manner for the more complex steels. Similar considerations will apply in the case where the treatment by diffusion is effected on two surfaces or on all the surface of the steel objects, in one, two or more times, these operations alternating with thermic treatment (temperings and the like) or suitable mechanical operations which may vary for each case according to the nature of the steel started with and of the steel obtained.

The operation above referred to may be applied directly to the mass of homogeneous steel as cast, or to the mass already brought to the desired shape by the ordinary mechanical manipulations, (hammering, rolling, pressing and the like). In every case, however, it would almost always be necessary to follow the chemical treatment described above by a suitable thermic treatment. But it is in the temper of the metallic pieces where the greatest advantages

of this method of manufacture and the superiority of the pieces produced in this manner are evident as compared with those obtained by the other methods. As a matter of fact by employing this method any given composition for the various zones of the piece of steel can be obtained and consequently the various parts of the object may be given the most suitable composition to be obtained whereby through a homogeneous tempering and applied to the whole, each part acquires the physical, chemical or mechanical properties (such as magnetic properties, resistance to chemical agents, hardness, plasticity, elasticity and the like) the most suitable for the purposes for which the piece has to be utilized. By this method armor plates for example, can be obtained which after one or more homogeneous and total temperings effected under the desired conditions of temperature and the like, possess mechanical properties (hardness, tenacity, and the like) differing in their various layers so that they can be most suitably adapted to the most varied uses.

Let us suppose for example to have to treat a special nickel steel showing the following composition: nickel 2.20%; carbon 0.10%; manganese 0.42%; silicon 0.30%; sulfur 0.04%; phosphorus 0.02%, and that it be intended to obtain a zone of 3 mm. thickness, in which the percentage of carbon should vary from 0.9% (on the outer face) down to 0.4% at 3 mm. depth, while the percentage of manganese, namely of the metal to be introduced by diffusion according to the present invention, should vary between 3% (on the outer face) and 0.7% at 3 mm. depth. In order to obtain this result it will be sufficient to heat the steel piece in contact with a granular mixture consisting of three parts of charcoal, one of finely pulverized manganese dioxide and one of barium carbonate. A temperature of 1150 degrees C. is to be kept up during about half of an hour; whereupon the same is to be allowed to gradually drop down to 700 degrees C. at the end of the three hours. In making these statements, as to the duration of the heating, it has been assumed that the time begins to run since the full heat has been laid on the steel pieces; the additional time necessary for reaching the aforesaid temperatures as well as for cooling after each treatment, of course depends upon the size of the pieces and the arrangement of the heating furnaces.

Having now particularly described and ascertained the nature of my said invention and in what manner the same is to be performed, I declare that what I claim is:

1. The process of forming steel plates or other articles, consisting in subjecting one or more surfaces of the article to contact with a certain characteristic metal steel

component, and at the same time to a material capable of varying the proportion of carbon in the article, for a considerable period of time and at a temperature regulated 5 to cause diffusion into the article for a considerable distance to form a zone in the article in which the percentage of the component metal united with the steel is graded from a maximum to a minimum and in 10 which zone the proportion of carbon is varied from the original quantity.

2. The process of forming steel plates or other articles, consisting in subjecting one or more surfaces of the article to contact 15 with a certain characteristic metal steel component and to a suitable decarbonizing material for a considerable period of time and at a temperature sufficient by itself to cause diffusion into the article for a considerable distance to form a zone in the article in which the percentage of the component metal united with the steel is graded from a maximum inwardly to a minimum and in 20 which zone the proportion of carbon in 25 the said zone is less than the original quantity.

3. The process of forming steel plates or other articles consisting in subjecting one or more surfaces of the article to contact with 30 a certain characteristic metallic steel component, for a considerable period of time and at a temperature between that of the

highest critical point of the steel employed and a temperature near its point of fusion whereby to cause diffusion into the article 35 for a considerable distance to form a zone in the article in which the percentage of the component metal united with the steel is graded from a maximum inwardly to a minimum. 40

4. The process of forming steel plates or other articles consisting in subjecting one or more surfaces of the article to contact with a certain characteristic metal steel component, and at the same time to a material capable of varying the proportion of carbon in the article, for a considerable period of time and at a temperature between that of the highest critical point of the steel employed and a temperature near its point of 45 fusion whereby to cause diffusion into the article for a considerable distance to form a zone in the article in which the percentage of the component metal united with the steel is graded from a maximum to a minimum and in 50 which zone the proportion of carbon is varied from the original quantity. 55

In testimony whereof I affix my signature in presence of two witnesses.

FEDERICO GIOLITTI. [L. S.]

Witnesses:

G. B. ZANARDO,  
ERNEST SANTI.